

# United States Patent [19]

Cole et al.

[11] 3,741,279

[45] June 26, 1973

[54] **METHOD OF CASTING**

[76] Inventors: Gerald S. Cole, 4839 Middlesex, Dearborn, Mich. 48126; Gustaf F. Bolling, 24646 Winona Drive, Dearborn, Mich. 48124

[22] Filed: Oct. 4, 1971

[21] Appl. No.: 186,336

**Related U.S. Application Data**

[63] Continuation-in-part of Ser. No. 760,126, Sept. 13, 1968, Pat. No. 3,614,976.

[52] U.S. Cl. .... 164/114, 164/122, 164/260

[51] Int. Cl. .... B22d 13/00

[58] Field of Search ..... 164/71, 83, 114-116, 164/122, 260

[56] **References Cited**

UNITED STATES PATENTS

1,010,851 12/1911 Bruckmann ..... 164/260  
1,040,517 10/1912 Crawford ..... 164/115

|           |         |                |           |
|-----------|---------|----------------|-----------|
| 2,116,367 | 5/1938  | Smith .....    | 164/260 X |
| 3,414,045 | 12/1968 | Harvey .....   | 164/116   |
| 3,568,752 | 3/1971  | Williams ..... | 164/114   |

**FOREIGN PATENTS OR APPLICATIONS**

399,331 10/1933 Great Britain ..... 164/71

*Primary Examiner*—R. Spencer Annear  
*Attorney*—Keith L. Zerschling et al.

[57]

**ABSTRACT**

This invention relates to a founding process involving metal alloy compositions which upon solidification precipitate at least two distinct phases simultaneously. The metallurgical structure of castings resulting from this founding process is altered by subjecting the solidifying metal to a mild angular or rotative acceleration. The direction of this angular acceleration is periodically reversed to avoid high rotational speeds. This results in an angular or rotative oscillation.

4 Claims, 5 Drawing Figures

*AS CAST STRUCTURE IN A GREY IRON*



CONVENTIONAL



OSCILLATED

3.3C + 3.1Si

1.5 TIMES

PATENTED JUN 26 1973

3,741,279

SHEET 1 OF 5

AS CAST STRUCTURE IN A GREY IRON



CONVENTIONAL

OSCILLATED

1.5 TIMES

FIG. 1

3.3C + 3.1Si

PATENTED JUN 26 1973

3,741,279

SHEET 2 OF 5



FIG. 2

FLAKE GRAPHITE STRUCTURE: THERE IS A PRONOUNCED REFINEMENT OF THE FLAKE STRUCTURE IN THE OSCILLATED INGOT.

SHEET 3 OF 5



B



(20 TIMES)

REMELTED NODULAR (I)

FIG. 3

FLAKE GRAPHITE STRUCTURE: LARGE EUTECTIC CELLS IN THE CONVENTIONALLY CAST INGOT ARE REORIENTED IN THE OSCILLATED INGOT.

PATENTED JUN 26 1973

3,741,279

SHEET 4 OF 5

FIG. 4



QUANTITATIVE METALLOGRAPHIC ANALYSIS OF PERCENT  
GRAPHITE IN A 4.1C, 1.6Si GREY CAST IRON.

PATENTED JUN 26 1973

3,741,279

SHEET 5 OF 5

FIG. 5

TRW VI A ALLOY



FORD 406 ALLOY



QUANTITATIVE METALLOGRAPHIC ANALYSIS OF PERCENT  
GAMMA PRIME IN TWO NICKEL-BASE SUPERALLOYS

### METHOD OF CASTING

This invention is a continuation in part of Application Ser. No. 760,126 filed Sept. 13, 1968 and now U.S. Pat. No. 3,614,976 issued Oct. 26, 1971.

### THE INVENTION

The origins of the founding art are lost in the mists of time and it has long been known that the final properties of castings are strongly influenced by the combined effects of many gross factors and also by many subtle factors such as metal composition, melting conditions, degree of superheat, inoculation, mold composition and rate of cooling. These sundry and subtle variables have been manipulated in many ways to obtain the desired final properties.

This invention is predicated upon our discovery that the metallurgical characteristics of castings which precipitate at least two distinct phases upon solidification can be decidedly improved by imparting to the solidifying casting an angular acceleration. This angular acceleration is obtained by rotating the solidifying casting first in one direction and then the other. This results in a continuous angular acceleration which varies also in sign and magnitude. Typical commercially important metals upon which this invention has been successfully practiced are gray irons and heat resistant super alloys based upon iron, nickel or cobalt. This invention is particularly applicable to castings whose surfaces are surfaces of revolution.

The velocity of rotation employed in the current process is not to be confused with the much greater velocity of rotation conventionally employed in the process known as centrifugal casting. Such a conventional centrifugal casting process is taught by a patent issued Oct. 27, 1942 to S. M. Stoddy et al. as 2,299,860. This patent teaches the production of an aircraft supercharger wheel from heat and corrosion resistant alloys and of approximately the same size as described later in the current invention. Stoddy states in line 46 of page 3 that the rate of rotation is 1,500 R.P.M. This is to be contrasted with the 100 R.P.M. which has been found to be adequate for the execution of Applicants' process. Inasmuch as the centrifugal forces vary as the square of the peripheral speed divided by the radius, the Stoddy process which is typical of commercial practice would subject the metal to stresses 225 times as great as those employed by Applicants.

This invention was carried out by casting the various metals into refractory molds supported upon a rotatable metal plate. This plate is driven by a reversible electric motor arranged to rotate the mold supporting plate at 120 R.P.M. when energized and permitted to come to full speed.

The oscillatory motion was obtained by reversing the electric motor each 4 seconds. This time interval is too brief to permit the metal plate to reach the full equilibrium speed of 120 R.P.M. and caused it to reverse in torque when a speed of only about 100 R.P.M. had been reached.

The tremendous commercial importance of gray iron made it a logical candidate upon which to demonstrate this invention. To this end FIGS. 1, 2 and 3 have been presented showing a conventional gray iron composition at varying degrees of magnification after casting during oscillation.

FIG. 1 is a conventional gray iron consisting essentially of iron alloyed with 3.3 percent carbon and 3.1

percent silicon. The magnification in FIG. 1 is only 1.5X but the radical change produced by oscillation is readily apparent.

FIG. 2 is the same alloy as FIG. 1 with the magnification increased to 30X. There is a pronounced refinement of the flake structure in the oscillated ingot as compared to the conventionally cast ingot.

FIG. 3 is a logical extension of the showings of FIGS. 1 and 2 and demonstrates the effect of oscillation upon a remelted conventional nodular iron. The large eutectic cells in the conventionally cast ingot are reoriented in the oscillated ingot. The magnification is 20X.

FIG. 4 constitutes a graphic presentation of the effect of oscillation upon the graphite distribution in a gray cast iron containing 4.1 percent carbon and 1.6 percent silicon. This drawing contains three curves, one each for the static mode of casting, for the rotated casting and for the oscillated casting. The abscissae represent the distance from the edge of the casting and the ordinates the volume percent graphite.

FIG. 5 is analogous to FIG. 4 except that it is directed to two nickel base super alloys known to the trade as TRW VI A alloy and Ford 406 alloy. The chemistry of these alloys is as follows:

|    | TRW VI A | Ford 406 |
|----|----------|----------|
| 25 | 6.1 Cr   | 6.0 Cr   |
|    | 7.5 Co   | 10.0 Co  |
|    | 2.0 Mo   | 1.0 Mo   |
|    | 5.8 W    | 8.5 W    |
|    | 5.4 Al   | 4.5 Al   |
|    | 1.0 Ti   | 2.0 Ti   |
|    | 0.5 Nb   | 2.0 Nb   |
|    | 9.0 Ta   | 6.0 Ta   |
|    | 0.13 C   | 0.13 C   |
|    | 0.015 B  | 0.015 B  |
|    | 0.1 Zr   | 0.1 Zr   |
|    | 0.5 Re   |          |
|    | 0.4 Hf   |          |

The pronounced effect of the oscillation upon the average percentage of primary gamma prime is readily apparent.

We claim as our invention:

1. In a method for controlling micro-structural phase concentrations in centrifugally cast metallic material, the steps of: subjecting a molten mass of said material to oscillations at least equal to about 4 seconds in period determined from the start of motion in one direction for each oscillation to the completion of motion in said one direction, the speed of said mass varying continuously during each oscillation and attaining an angular speed no greater than about 100 r.p.m. near the terminal portion of each oscillatory movement.

2. The method as in claim 1, in which the molten mass is comprised of iron alloyed with at least 3.3 percent carbon and about 1.6 percent silicon, the oscillatory movement of said mass producing a generally uniform distribution of a graphite phase in cast iron, the uniform distribution being viewed from the outer to the most inner regions of the casting.

3. The method as in claim 1, in which the molten mass is comprised of a nickel base super alloy comprising about 6% Cr, 7% Co, 2% Mo, 5.4% Al, 9.0% Ta, 5.8% W, the oscillatory movement of said mass producing a casting in which the primary gamma prime phase is generally uniform throughout the entire casting with a cross-sectional variation no greater than 1 percent.

4. The method as in claim 1, in which the molten mass is comprised of a nickel based alloy having at least 6% C, about 10% Co and about 1% Mo, 8.5% W, 4.5% Al, the oscillatory movement of said mass producing a casting in which a primary gamma prime phase is predominantly concentrated at a mid-radial region of said casting, the primary gamma prime phase having a concentration at said mid-radial region at least 1 percent greater than the concentration at either the innermost or outermost region of said casting.

\* \* \* \* \*